# EUROPEAN PATENT SPECIFICATION

(11) **EP 1 631 694 B1**
(45) Date of publication and mention of the grant of the patent: **15.04.2009**
(21) Application number: 04752554.8
(22) Date of filing: 18.05.2004
(51) Int. Cl.: C22C 29/06, B22F 7/00

(54) **EROSION-CORROSION RESISTANT CARBIDE CERMETS FOR LONG TERM HIGH TEMPERATURE SERVICE**
EROSION- UND KORROSIONBESTÄNDIGE KARBIDCERMETS FÜR HOCHTEMPERATURANWENDUNGEN
CERMETS A BASE DE CARBURE RESISTANT A L'EROSION ET A LA CORROSION POUR UTILISATION DE LONGUE DUREE AUX TEMPERATURES ELEVEES

(30) Priority: 20.05.2003 US 471789 P; 22.04.2004 US 829823
(43) Date of publication of application: 08.03.2006
(73) Proprietor: ExxonMobil Research and Engineering Company, Annandale NJ 08801-0900 (US)
(72) Inventor: BANGARU, Narasimha-Rao, Venkata, Pittstown NJ 08867 (US); CHUN, ChangMin, Belle Mead, NJ 08502 (US); THIRUMALAI, Neeraj, Srinivas, Phillipsburg, NJ 08865 (US); LING, Shiun, Washington, NJ 07882 (US); JIN, Hyun-Woo, Easton PA 18040 (US); KOO, Jayoung, Y., Somerset NJ 08873 (US); PETERSON, John, Roger, Ashburn, VA 20147 (US); ANTRAM, Robert, Lee, Warrenton, VA 20186 (US); FOWLER, Christopher, John, Springfield, VA 22150 (US)
(74) Representative: Mareschal, Anne
(86) International application number: PCT/US2004/015558
(87) International publication number: WO 2004/104250

(56) References cited:
- EP-A- 0 482 831
- EP-A- 0 641 869
- WO-A-83/01917
- US-A- 4 173 457
- PATENT ABSTRACTS OF JAPAN vol. 2000, no. 15, 6 April 2001 (2001-04-06) -& JP 2000 345314 A (TOCALO CO LTD), 12 December 2000 (2000-12-12)

## Description

### FIELD OF INVENTION

The present invention relates to cermet compositions. More particularly the invention relates to chromium carbide containing cermet compositions and their use in high temperature erosion and corrosion applications.

### BACKGROUND OF INVENTION

Abrasive and chemically resistant materials find use in many applications where metal surfaces are subjected to substances which would otherwise promote erosion or corrosion of the metal surfaces.

Reactor vessels and transfer lines used in various chemical and petroleum processes are examples of equipment having metal surfaces that often are provided with materials to protect the surfaces against material degradation. Because these vessels and transfer lines are typically used at high temperatures protecting them against degradation is a technological challenge. Currently refractory liners are used to protect metal surfaces exposed at high temperature to erosive or corrosive environments. The lifespan of these refractory liners, however, is significantly limited by mechanical attrition of the liner, especially when exposed to high velocity particulates, often encountered in petroleum and petrochemical processing. Refractory liners also commonly exhibit cracking and spallation. Thus, there is a need for liner material that is more resistant to erosion and corrosion at high temperatures.

Ceramic metal composites or cermets are known to possess the attributes of the hardness of ceramics and the fracture toughness of metal but only when used at relatively moderate temperatures, for example, from 25°C to no more than about 300°C. Tungsten carbide (WC) based cermets, for example, have both hardness and fracture toughness making them useful in high wear applications such as in cutting tools and drill bits cooled with fluids. WC based cermets, however, degrade at sustained high temperatures, greater than about 600°F (315°C).

Chromium carbide has been a potentially suitable ceramic phase for use in cermets because its three crystallographic forms: the cubic (Cr₂₃C₆) the hexagonal (Cr₇C₃) and the orthorhombic (Cr₃C₂) have excellent oxidation resistance at elevated temperatures; yet cermets formed from these carbides typically undergo transformations at elevated temperatures which result in the formation of microstructural phases which have a deleterious effect on the properties of such cermets. EP-A-0 641 869 relates to powders for use in spray-coating, comprising particles containing of metal carbide core (containing Cr₃C₂) and Ni-Cr alloys.

The object of the present invention is to provide new and improved cermet compositions.

Another object of the invention is to provide chromium carbide containing cermet compositions suitable for use at high temperatures.

Another object of the invention is to provide chromium carbide containing cermet compositions with long term microstructural stability suitable for long term service at high temperatures.

Yet another object of the invention is to provide an improved method for protecting metal surfaces against erosion and corrosion under high temperature conditions.

These and other objects will become apparent from the detailed description which follows.

Broadly stated, the present invention is a cermet composition comprising a chromium carbide ceramic phase dispersed in a binder phase. The ceramic phase which constitutes about 50 vol% to about 95 vol% of the total volume of the cermet composition is a chromium carbide selected from the group consisting of Cr₂₃C₆, Cr₇C₃, and mixtures thereof.

The binder phase is selected from the group consisting of (i) alloys containing about 60 wt% to about 98 wt% Ni; about 2 wt% to about 35 wt% Cr; and up to 5 wt% of an element selected from the group consisting of Al, Si, Mn, Ti and mixtures thereof; and (ii) alloys containing about 0.01 wt% to about 35 wt% Fe; about 25 wt% to about 97.99 wt% Ni, about 2 wt% to about 35 wt% Cr; and up to about 5 wt% of an element selected from the group consisting of Al, Si, Mn, Ti and mixtures thereof, the wt% in each instance based on the total weight of the alloy.

This and other embodiment of the invention, including where applicable those preferred, will be elucidated in the detailed description which follows.

### BRIEF DESCRIPTION OF THE FIGURES

Figure 1 is a scanning electron microscopy (SEM) image of the surface of a cermet made with an initial Cr₃C₂ in 30 vol% Ni-20 Cr binder. Ni-20 Cr indicates 80 wt% Ni and 20 wt% Cr.

Figure 2 is a SEM image of the surface of a cermet made with an initial Cr₇C₃ in 30 vol% Ni-20 Cr binder.

Figure 3 is a SEM image of the surface of a cermet made with an initial Cr₂₃C₆ in a 30 vol% Ni-20 Cr binder.

Figure 4 is a SEM image of the surface of a cermet made with an initial Cr₃C₂ in a 30vol% 304 stainless steel (304SS) binder after exposure to 800°C for 1000 hours.

### DETAILED DESCRIPTION OF THE INVENTION

In one embodiment the invention is a cermet composition comprising a chromium carbide ceramic phase dispersed in a continuous binder phase.

The ceramic phase constitutes about 50 vol% to about 95 vol% of the total volume of the cennet composition, the ceramic phase being a chromium carbide selected from the group consisting of Cr₂₃C₆, Cr₇C₃, and mixtures thereof, where this group is intended to include sub and super stoichiometric variances thereof.

The particle size diameter of the ceramic phase typically is below about 3 mm, preferably below about 100µm and more preferably below about 50µm. The dispersed ceramic particles can be any shape. Some non-limiting examples include spherical, ellipsoidal, polyhedral, distorted spherical, distorted ellipsoidal and distorted polyhedral shaped. By particle size diameter is meant the measure of longest axis of the 3-D shaped particle. Microscopy methods such as optical microscopy (OM), scanning electron microscopy (SEM) and transmission electron microscopy (TEM) can be used to determine the particle sizes.

The binder phase is selected from the group consisting of (i) alloys containing about 60 wt% to about 98 wt% Ni; about 2 wt% to about 35 wt% Cr; and up to about 5 wt% of an element selected from the group consisting of Al, Si, Mn, Ti and mixtures thereof; and (ii) alloys containing about 0.01 wt% to about 35 wt% Fe; about 25 wt% to about 97.99 wt% Ni, about 2 wt% to about 35 wt% Cr; and up to about 5 wt% of an element selected from the group consisting of Al, Si, Mn, Ti and mixtures thereof, the wt% in each instance based on the total weight of the alloy.

Illustration of cermet compositions suitable for use at elevated temperatures include:
(1) about 50 vol% Cr₇C₃ in a binder comprising 78 wt% Ni, about 4 wt% Fe and 18 wt% Cr;
(2) about 70 vol% Cr₇C₃ in a binder comprising 78 wt% Ni, about 4 wt% Fe and 18 wt% Cr;
(3) about 94 vol% Cr₇C₃ in a binder comprising 75 wt% Ni, about 7 wt% Fe, and about 18 wt% Cr;
(4) about 50 vol% Cr₂₃C₆ in a binder comprising 72wt% Ni, about 10 wt% Fe, and 18 wt% Cr;
(5) about 50 vol% Cr₂₃C₆ in a binder comprising 67 wt% Ni, 15 wt% Fe and 18 wt% Cr; and
(6) about 90 vol% Cr₂₃C₆ in a binder comprising 77 wt% Ni, 5 wt% Fe and 18 wt% Cr.

Preferred cermet compositions are the follows:
(1) 50 vol% to 90 vol% Cr₂₃C₆ in binder (i); and
(2) 50 vol% to 90 vol% Cr₇C₃ in binder (i).

The cermet compositions are made by general powder metallurgical techniques such as mixing, milling, pressing, sintering and cooling, employing as starting materials a chromium carbide ceramic powder and a binder powder in the volume ratio of 50:50 to 95:5 respectively. Preferably the chromium carbide powder is one Cr₂₃C₆ or Cr₇C₃, although mixtures of these may be used. Preferably the binder is one of the alloy compositions set forth in Table 1.

**Table 1**

| Alloy Type | Composition (wt%) |
|---|---|
| NiCr | Bal Ni:20 Cr |
| NiCrSi | Bal Ni:20.1 Cr:2.0 Si:0.4 Mn:0.09 Fe |
| FeNiCr | Bal Fe:> 12 Cr > 36 Ni |

| | |
|---|---|
| Bal = Balance | |

These powders are milled in a ball mill in the presence of a sufficient amount of an organic liquid such as ethanol for a time sufficient to substantially disperse the powders in each other. The liquid is removed and the milled powder is dried, placed in a die and pressed into a green body. The green body is then sintered at temperatures above about 1200°C up to about 1600°C for times ranging from about 10 minutes to about 4 hours. The sintering operation is preferably performed in an inert atmosphere or a reducing atmosphere or under vacuum. For instance, the inert atmosphere can be argon and the reducing atmosphere can be hydrogen. Thereafter the sintered body is allowed to cool, typically to ambient conditions. The cermet production according to the process described herein allows fabrication of bulk cermet bodies exceeding 5 mm in thickness.

These processing conditions result in the dispersion of the carbide or carbides in the binder. Additionally, the processing results in some compositional changes in the ceramic and binder. For example, when the ceramic employed is Cr₂₃C₆ in the same binder there is substantially no change in the composition of the ceramic.

The volume percent of cermet phase (and cermet components) excludes pore volume due to porosity. The cermet can be characterized by a porosity in the range of 0.1 to 15 vol%. Preferably, the volume of porosity is 0.1 to less than 10% of the volume of the cermet. The pores comprising the porosity is preferably not connected but distributed in the cermet body as discrete pores. The mean pore size is preferably the same or less than the mean particle size of the chromium carbide ceramic phase.

One feature of the cermets of the invention is their long term microstructural stability, even at elevated temperatures, making them particularly suitable for use in protecting metal surfaces against erosion at temperatures in the range of about 300°C to about 1000°C. This stability permits their use for prolonged time periods, for example greater than 2 years. In contrast many known cernets undergo transformations at elevated temperatures which result in the formation of phases which have a deleterious effect on the properties of the cermet.

The long term microstructural stability of the cermets of the instant invention was confirmed by computational thermodynamics using calculation of phase diagram (CALPHAD) methods known to one of ordinary skill in the art of computational thermodynamic calculation methods. These calculations confirmed that the various carbide phases, their amounts, the binder amount and the respective chemistries lead to cermet compositions with long term microstructural stability. Further, lab experiments were conducted in which the cermet compositions of the instant invention were exposed at 800°C for 1000 hours in air. Analysis of the bulk microstructure of the resultant cermet after this 1000h high temperature exposure showed that the starting microstructure was substantially preserved as determined by SEM.

The cermet compositions of the instant invention can exhibit long term microstructural stability lasting at least 25 years when exposed to temperatures up to 1000°C.

Another feature of the cermets of this invention is that they have fracture toughness of greater than about 3 MPa·m^{1/2}, preferably greater than about 5 MPa·m^{1/2}, and most preferably greater than about 10 MPa·m^{1/2}. Fracture toughness is the ability to resist crack propagation in a material under monotonic loading conditions. Fracture toughness is defined as the critical stress intensity factor at which a crack propagates in an unstable manner in the material. Loading in three-point bend geometry with the pre-crack in the tension side of the bend sample is preferably used to measure the fracture toughness with fracture mechanics theory. The binder phase of the cermet of the instant invention as described in the earlier paragraphs is primarily responsible for imparting this attribute.

The high temperature stability of the cermets of the invention makes them suitable for applications where refractories are currently employed. A non-limiting list of suitable uses include liners for process vessels, transfer lines, cyclones, for example, fluid-solids separation cyclones as in the cyclone of Fluid Catalytic Cracking Unit used in refining industry, grid inserts, thermo wells, valve bodies, side valve gates and guides catalyst regenerators, and the like. Thus, metal surfaces exposed to erosive or corrosive environments, especially at about 300°C to about 1000°C are protected by providing the surface with a layer of the ceramic compositions of the invention. The cermets of the instant invention can be affixed to metal surfaces by mechanical means or by welding.

### Determination of Volume Percent:

The volume percent of each phase, component and the pore volume (or porosity) were determined from the 2-dimensional area fractions by the Scanning Electron Microscopy method. Scanning Electron Microscopy (SEM) was conducted on the sintered cermet samples to obtain a secondary electron image preferably at 1000x magnification. For the area scanned by SEM, X-ray dot image was obtained using Energy Dispersive X-ray Spectroscopy (EDXS). The SEM and EDXS analyses were conducted on five adjacent areas of the sample. The 2-dimensional area fractions of each phase was then determined using the image analysis software: EDX Imaging/Mapping Version 3.2 (EDAX Inc, Mahwah, New Jersey 07430, USA) for each area. The arithmetic average of the area fraction was determined from the five measurements. The volume percent (vol%) is then determined by multiplying the average area fraction by 100. The vol% expressed in the examples have an accuracy of +/-50% for phase amounts measured to be less than 2 vol% and have an accuracy of +/-20% for phase amounts measured to be 2 vol% or greater.

### Determination of weight percent:

The weight percent of elements in the cermet phases was determined by standard EDXS analyses.

The following non-limiting examples are included to further illustrate the invention.

### EXAMPLE 1 (comparative)

70 vol% of 14.0µm average diameter of Cr₃C₂ powder (99.5% purity, from Alfa Aesar) and 30 vol% of Ni-20Cr alloy binder powder (Alfa Aesar, screened below 325 mesh) were dispersed with ethanol in high density polyethylene milling jar. The powders in ethanol were mixed for 24 hours with yttria toughened zirconia balls (10 mm diameter, from Tosoh Ceramics) in a ball mill at 100 rpm. The ethanol was removed from the mixed powders by heating at 130°C for 24 hours in a vacuum oven. The dried powder was compacted in a 40 mm diameter die in a hydraulic uniaxial press (SPEX 3630 Automated X-press) at 5,000 psi. The resulting green disc pellet was ramped up to 400°C at 25°C/min in argon and held for 30 min for residual solvent removal. The disc was then heated to 1450°C at 15°C/min in argon and held at 1450°C for 1 hour. The temperature was then reduced to below 100°C at -15°C/min.

The resulting cermet comprises:
i) 63 vol% Cr₃C₂ with average grain size of 20 µm
ii) 12 vol% Cr₇C₃ with average grain size of 20 µm
iii) 25 vol% Cr-depleted alloy binder (87Ni:13Cr in wt%).

Figure 1 is a SEM image of the cermet processed according to this example, wherein the bar represents 20µm. In this image the chromium carbide phase appears light and the binder phase appears dark.

### EXAMPLE 2

The mixing and pressing procedures of Example 1 was followed using 70 vol% of 14.0µm average diameter of Cr₇C₃ powder (99.5% purity, from Alfa Aesar) and 30 vol% of Ni-20Cr alloy binder powder (Alfa Aesar, screened below 325 mesh). The disc was then heated to 1400°C for 1 hour at 15°C/min in hydrogen. The temperature was then reduced to below 100°C at -15°C/min.

The resulting cermet comprised:
i) 67 vol% Cr₇C₃ with average grain size of 20µm
ii) 33 vol% Cr-enriched alloy binder (76Ni:24Cr in wt%).

Figure 2 is a SEM image of the cermet processed according to this example, wherein the bar represents 20µm. In this image the chromium carbide phase appears light and the binder phase appears dark.

### EXAMPLE 3

The procedure of Example 2 was followed using 70 vol% of 14.0µm average diameter of Cr₂₃C₆ powder (99.5% purity, from Alfa Aesar) and 30 vol% of Ni-20Cr alloy binder powder (Alfa Aesar, screened below 325 mesh).

The result cermet comprised of:
i) 67 vol% Cr₂₃C₆ with average grain size of 20µm
ii) 33 vol% Cr-enriched alloy binder (69Ni:31Cr in wt%).

Figure 3 is a SEM image of the cermet processed according to this example, wherein the bar represents 20µm. In this image the chromium carbide phase appears light and the binder phase appears dark.

### EXAMPLE 4 (comparative)

The procedure of Example 2 was followed using 85 vol% of 14.0µm average diameter of Cr₃C₂ powder (99.5% purity, from Alfa Aesar) and 15 vol% of Ni-20Cr alloy binder powder (Alfa Aesar, screened below 325 mesh).

During heating, some Cr₃C₂ phase is replaced by Cr₇C₃ phase. As result, carbide volume fraction increases and Cr content is depleted in the binder. The result cermet comprised of:
i) 80 vol% Cr₃C₂ with average grain size of 20µm
ii) 7 vol% Cr₇C₃ with average grain size of 20µm
iii) 13 vol% Cr-depleted alloy binder (85Ni:15Cr in wt%).

### EXAMPLE 5

The cermet compositions of examples 1,2 and 3were exposed in air at 800°C for 1000 hours in a Lindberg box furnace. After exposure the samples were analyzed using SEM. No significant precipitation of new phases, change in the proportion of the original phase composition or change in the respective chemistry was observed in any of the 3 aforestated samples. Thus the cermet composition of example 1, 2 and 3 were determined to possess long term microstructural stability.

### EXAMPLE 6 (COMPARATIVE EXAMPLE)

A comparative example of a system that does not form a preferred thermodynamically stable cermet is prepared using the procedure of Example 1 and 70 vol% of 14.0µm average diameter of Cr₃C₂ powder (99.5% purity, from Alfa Aesar) and 30 vol% of 6.7µm average diameter 304SS alloy binder powder (Osprey Metals, Fe(balance):18.5Cr:9.6Ni:1.4Mn:0.63Si, 95.9% screened below -16µm). The disc was then heated to 1400°C at 15°C/min in argon and held at 1400°C for 1 hour. During heating, a significant vol% of Cr₃C₂ phase is replaced by Cr₇C₃ phase. As net result, carbide volume fraction increases and Cr content is depleted in the binder.

The result cermet comprised of the non-equilibrium microstructure:
i) 8 vol% Cr₃C₂ with average grain size of 20µm
ii) 72 vol% Cr₇C₃ with average grain size of 20µm
iii) 20 vol% Cr-depleted alloy binder

Next, the sintered disc was heated in air at 800°C for 1000 hours. After exposure to 800°C in air for 1000 hours this cermet comprises:
i) >9.5 vol% Cr₃C₂
ii) >85.5 vol% Cr₇C₃
iii) <5 vol% Cr-depleted alloy binder (13.2Si:9.4Cr:8.9Fe:68.5Ni in wt%).

Figure 4 is a SEM image of the cermet after heating in air according to this example, wherein the bar represents 10µm. In this image the chromium carbide phase appears light and the binder phase appears dark. This figure shows < 5 vol% 304SS and > 95 vol% chrome carbides after this relative short-term exposure to high temperature. The metal composition has become depleted in chromium content thereby decreasing the fracture toughness of the cermet.

### EXAMPLE 7

Each of the cermets of Examples 1 to 4 was subjected to a hot erosion and attrition test (HEAT) and was found to have an erosion rate of less than 1.0x10⁻⁶ cc/gram SiC erodant. The procedure employed was as follows:
1) A specimen cermet disk of about 35 mm diameter and about 5 mm thick was weighed.
2) The center of one side of the disk was then subjected to 1200g/min of SiC particles (220 grit #1 Grade Black Silicon Carbide, UK abrasives, Northbrook, IL) entrained in heated air exiting from a tube with a 0.5 inch diameter ending at 1 inch from the target at an angle of 45°. The velocity of the SiC was 45.7 m/sec.
3) Step (2) was conducted for 7 hrs at 732°C.
4) After 7 hrs the specimen was allowed to cool to ambient temperature and weighed to determine the weight loss.
5) The erosion of a specimen of a commercially available castable refractory was determined and used as a Reference Standard. The Reference Standard erosion was given a value of 1 and the results for the cermet specimens are compared in Table 2 to the Reference Standard. In Table 2 any value greater than 1 represents an improvement over the Reference Standard.

**Table 2**

| Cermet {Example} | Starting Weight (g) | Finish Weight (g) | Weight Loss (g) | Bulk Density (g/cc) | Erodant (g) | Erosion (cc/g) | Improvement [(Normalized erosion)⁻¹] |
|---|---|---|---|---|---|---|---|
| Cr3C2 L 30 | 18.6737 | 15.0660 | 3.6077 | 7.350 | 5.04E+5 | 7.3766E-7 | 1.4 |
| NiCr {1} | | | | | | | |
| Cr7C3 L 30 | 23.6681 | 21.0301 | 2.6380 | 7.360 | 5.34E+5 | 6.7121E-7 | 1.6 |
| NiCr {2} | | | | | | | |
| Cr23C6 L | 23.5976 | 21.6016 | 1.9960 | 7.350 | 5.04E+5 | 5.3882E-7 | 1.9 |
| 30 NiCr {3} | | | | | | | |
| Cr3C2 L 15 | 19.6071 | 17.6609 | 1.9462 | 7.090 | 5.04E+5 | 5.4464E-7 | 1.9 |
| NiCr {4} | | | | | | | |

### EXAMPLE 8

Each of the cermets of Examples 1 to 4 was subjected to a corrosion test and found to have a corrosion rate less than about 1.0x10⁻¹¹ g²/cm⁴s. The procedure employed was as follows:
1) A specimen cermet of about 10 mm square and about 1 mm thick was polished to 600 grit diamond finish and cleaned in acetone.
2) The specimen was then exposed to 100 cc/min air at 800°C in thermogravimetric analyzer (TGA).
3) Step (2) was conducted for 65 hours at 800°C.
4) After 65 hours the specimen was allowed to cool to ambient temperature.
5) Thickness of oxide scale was determined by cross sectional microscopy examination of the corrosion surface.
6) All the thickness of oxide scale formed on specimen surface was less than 1 µm, representing superior corrosion resistance.

## Claims

1. A cermet composition comprising a chromium carbide ceramic phase dispersed in a binder phase, said cermet composition comprising:
(a) 50 vol% to 95 vol%, based on the total volume of the cermet composition, of a ceramic phase, wherein the ceramic phase being a chromium carbide selected from the group consisting of Cr₂₃C₆, Cr₇C₃ and mixtures thereof; and
(b) the balance of the vol%, based on the total volume of the cermet composition, of a binder phase selected from the group consisting of
(i) alloys containing, based on the total weight of the alloy, 60 wt% to 98 wt% Ni; 2 wt% to 35 wt% Cr; and up to 5 wt% of an element selected from the group consisting Al, Si, Mn, Ti and mixtures thereof; and
(ii) alloys containing 0.01 wt% to 35 wt% Fe; 25 wt% to 97.99 wt% Ni, 2wt% to 35 wt% Cr; and up to 5 wt% of an element selected from the group consisting of Al, Si, Mn, Ti and mixtures thereof.

2. The composition of claim 1 wherein the binder is (i).

3. The composition of claim 1, wherein the binder is (ii).

4. The composition of any of claims 1 to 3, wherein the chromium carbide is Cr₂₃C₆.

5. The composition of any of claims 1 to 3, wherein the chromium carbide is Cr₇C₃.

6. The composition of any of the preceding claims, wherein the ceramic phase is in the form of particles having a particle size diameter below 3 mm, preferably below 100 µm, more preferably below 50 µm.

7. The composition of any one of the preceding claims having a long term microstructural stability lasting at least 25 years when exposed at temperatures up to 1000°C.

8. A method for protecting a metal surface exposed to an erosive material at temperatures in the range of 300°C to 850°C, the method comprising providing the metal surface with a composition according to any of claims 1 to 7.

9. The method of claim 8 wherein said surface comprises the inner surface of a fluid-solids separation cyclone.

10. The composition of any of claims 1 to 7 or a method for protecting a metal surface according to any of claims 8 or 9, wherein the cermet composition is in the form of bulk cermet bodies exceeding 5 mm in thickness.

## Patentansprüche

1. Cermetzusammensetzung, die eine Chromcarbid-Keramikphase umfasst, die in einer Bindemittelphase dispergiert ist, wobei die Cermetzusammensetzung umfasst:
(a) 50 Vol.% bis 95 Vol.%, bezogen auf das Gesamtvolumen der Cermetzusammensetzung, einer Keramikphase, wobei die Keramikphase Chromcarbid ausgewählt aus der Gruppe bestehend aus Cr₂₃C₆, Cr₇C₃ und Mischungen davon ist,
(b) in den restlichen Vol.%, bezogen auf das Gesamtvolumen der Cermetzusammensetzung, eine Bindemittelphase ausgewählt aus der Gruppe bestehend aus:
(i) Legierungen, die, bezogen auf das Gesamtgewicht der Legierung, 60 Gew.-% bis 98 Gew.-% Ni, 2 Gew.-% bis 35 Gew.-% Cr und bis zu 5 Gew.-% eines Elements ausgewählt aus der Gruppe bestehend aus Al, Si, Mn, Ti und Mischungen davon enthalten, und
(ii) Legierungen, die 0,01 Gew.-% bis 35 Gew.-% Fe, 25 Gew.-% bis 97,99 Gew.-% Ni, 2 Gew.-% bis 35 Gew.-% Cr und bis zu 5 Gew.-% eines Elements ausgewählt aus der Gruppe bestehend aus Al, Si, Mn, Ti und Mischungen davon enthalten.

2. Zusammensetzung nach Anspruch 1, bei der das Bindemittel (i) ist.

3. Zusammensetzung nach Anspruch 1, bei der das Bindemittel (ii) ist.

4. Zusammensetzung nach einem der Ansprüche 1 bis 3, bei der das Chromcarbid C₂₃C₆ ist.

5. Zusammensetzung nach einem der Ansprüche 1 bis 3, bei der das Chromcarbid C₇C₃ ist.

6. Zusammensetzung nach einem der vorhergehenden Ansprüche, bei der die Keramikphase in Form von Partikeln mit einem Partikelgrößendurchmesser unter 3 mm, vorzugsweise unter 100 µm, insbesondere unter 50 µm vorliegt.

7. Zusammensetzung nach einem der vorhergehenden Ansprüche mit einer Langzeit-Mikrostrukturstabilität, die mindestens 25 Jahre anhält, wenn sie Temperaturen bis zu 1000°C ausgesetzt wird.

8. Verfahren zum Schützen einer Metalloberfläche, die bei Temperaturen im Bereich von 300°C bis 850°C einem erosiven Material ausgesetzt ist, bei dem die Metalloberfläche mit einer Zusammensetzung gemäß einem der Ansprüche 1 bis 7 versehen wird.

9. Verfahren nach Anspruch 8, bei dem die Oberfläche die Innenseite eines Fluid-Feststoff-Trennzyklons umfasst.

10. Zusammensetzung nach einem der Ansprüche 1 bis 7 oder Verfahren zum Schützen einer Metalloberfläche gemäß einem der Ansprüche 8 oder 9, bei dem die Cermetzusammensetzung in Form von Massencermetkörpern mit mehr als 5 mm Dicke vorliegt.

## Revendications

1. Composition de cermets comprenant une phase céramique à base de carbure de chrome dispersée dans une phase de liant, ladite composition de cermets comprenant :
(a) de 50 % en volume à 95 % en volume, basé sur le volume total de la composition de cermets, d'une phase céramique, dans laquelle la phase céramique est un carbure de chrome choisi parmi le groupe constitué du Cr₂₃C₆, du Cr₇C₃ et de mélanges de ceux-ci ; et
(b) le reste du % en volume, basé sur le volume total de la composition de cermets, est une phase d'un liant choisi parmi le groupe constitué
(i) d'alliages contenant, basé sur le poids total de l'alliage, de 60 % en poids à 98 % en poids de Ni, de 2 % en poids à 35 % en poids de Cr et jusqu'à 5 % en poids d'un élément choisi par le groupe constitué des atomes d'Al, de Si, de Mn et de Ti et de mélanges de ceux-ci ; et
(ii) d'alliages contenant de 0,01 % en poids à 35 % en poids de Fe, de 25 % en poids à 97,99 % en poids de Ni, de 2 % en poids à 35 % en poids de Cr et jusqu'à 5 % en poids d'un élément choisi par le groupe constitué des atomes d'Al, de Si, de Mn et de Ti et de mélanges de ceux-ci.

2. Composition selon la revendication 1, dans laquelle le liant est (i).

3. Composition selon la revendication 1, dans laquelle le liant est (ii).

4. Composition selon l'une quelconque des revendications 1 à 3, dans laquelle le carbure de chrome est le Cr₂₃C₆.

5. Composition selon l'une quelconque des revendications 1 à 3, dans laquelle le carbure de chrome est le Cr₇C₃.

6. Composition selon l'une quelconque des revendications précédentes, dans laquelle la phase céramique est sous la forme de particules dont la dimension est inférieure à 3 mm, de préférence inférieure à 100 µm, plus préférablement inférieure à 50 µm.

7. Composition selon l'une quelconque des revendications précédentes, dont la stabilité microstruturelle à long terme dure au moins 25 ans lorsqu'elle est exposée à des températures qui peuvent atteindre 1 000 °C.

8. Procédé de protection d'une surface métallique soumise à un matériau érosif à des températures dans la plage de 300 °C à 850 °C, le procédé comprenant la fourniture à la surface métallique d'une composition selon l'une quelconque des revendications 1 à 7.

9. Procédé selon la revendication 8, dans lequel ladite surface comprend la surface interne d'un cyclone de séparation fluide-solides.

10. Composition selon l'une quelconque des revendications 1 à 7 ou procédé de protection d'une surface métallique selon l'une des revendications 8 ou 9, dans lequel la composition de cermets est présente sous la forme d'un matériau de cermet en vrac dont l'épaisseur excède 5 mm.
